

March 20, 1934.

O. BUSSE

1,951,501

PROCESS FOR PRESSING METAL BLANKS

Filed Nov. 2, 1931



Fig.3.



Fig.2.



Fig.4.



Fig.1.

*Inventor*  
Otto Busse.

*by*  
W. E. Evans.  
*Attorney.*

## UNITED STATES PATENT OFFICE

1,951,501

## PROCESS FOR PRESSING METAL BLANKS

Otto Busse, Neheim-on-the-Ruhr, Germany

Application November 2, 1931, Serial No. 572,631  
In Germany November 7, 1930

1 Claim. (Cl. 207—10)

This invention relates to a method of extruding metal blanks in the form of bars, wires, bands and tubes, more especially by the use of a plunger press having a matrix disposed in front of a hollow plunger and penetrating into the receiver.

The metal must be extruded at a temperature determined according to the nature of the alloy, which temperature must be maintained. If the temperature of extrusion be too low the receiver and the matrix are exposed to too great a stress and the structure and the mechanical properties—particularly the expansibility of the product and its capacity for passing the notched bar test—are prejudicially affected. If the temperature of the blank is too high, the first part of the final product is rendered useless by the presence of transverse fractures and bubbles, while the steel receiver loses its strength, widens in bore, and become useless. The best, alloyed and improved steel for the receiver should not be heated theoretically to a temperature above 600° C.—in practice a temperature of 500° C. is not exceeded—as the steel loses its temper at this temperature. The best known and most used alloy, consisting of 58 to 60% of copper, 2% of lead and the remainder of zinc should be extruded at a temperature which is not below 720° C.

According to the invention the blank is heated to different temperatures from one end to the other, and is inserted into the receiver of the press in such manner that the colder end is extruded before the warmer end.

The excess temperature of the rear end of the blank must be such that the material flowing through the matrix is at the moment at the correct temperature for extrusion. The excess heat is transmitted to the matrix, the plunger and the receiver during the extrusion of the first part of the blank.

The accompanying drawing shows the known hydraulic press that is usually employed and which is provided with main pressure cylinder 10, matrix 11, hollow plunger 12 and receiver 13, with the blank to be extruded, which is conceived in this case as consisting of a metal cylinder, lying between the operative parts of the press, that is to say, between the main pressure cylinder 10 and the hollow plunger 12 provided with the matrix 11. The receiver 13 is then pushed over the blank and the extrusion operation begins. In the case, for example, of the alloy known as Ms 58 the blank 1 to be extruded is according to the present practice introduced at a working temperature of 730° to 750° C. In carrying out the invention the blank 1 is preheated at the forward end 2 to from

730° to 750° C.—that is, the usual temperature—while the rear end 3 is heated to a temperature of from about 800° to 820° C. This difference of temperature must, it will be understood, be selected according to the nature of the alloy, the rapidity of the extrusion operation, and the dimensions of the operative parts of the press, and therefore in accordance with the transference of heat from the blank to the press.

An advantage of the invention is,—in addition to the lengthening of the lift of the matrix and receiver, the saving in power and the obtaining of a perfect final product—an increase in the output of the press to about double. This increase in output is due to the fact that in the process according to the invention blanks of greater length and greater cross-section than those that are handled by known methods of production can be extruded.

The invention is not limited to the example hereinbefore described. It may be applied in similarly operated presses, for example, in plunger presses in which the matrix is fixed in front of the receiver, and, in such a press, particularly for the extrusion of tubes.

I claim:

A method of extruding metal blanks in the form of bars, wires, bands and tubes, by the use of a plunger press having a matrix disposed in front of a hollow plunger, consisting in heating the blank of the material to be extruded so that one end of the blank is at a higher temperature than the other end and in inserting the blank into the receiver of the press with the end at the higher temperature disposed farthest from the matrix, the said higher temperature being determined so that the metal at the far end of the blank is at approximately the correct temperature for extrusion when it is passing through the matrix.

OTTO BUSSE. 95

100

105

110